

## UNITED STATES PATENT OFFICE

2,096,797

## COLORATION OF MATERIALS

George Holland Ellis, Spordon, near Derby, England, assignor to Celanese Corporation of America, a corporation of Delaware

No Drawing. Application May 4, 1932, Serial No. 609,271. In Great Britain May 22, 1931

8 Claims. (Cl. 8—5)

This invention relates to a new process of producing pattern effects on textile materials, and to the production of compounds or compositions suitable for use in this process.

5 In order to produce pattern effects on textile materials the latter may be colored with a ground color and then printed with a composition containing an agent which will discharge that color in the selected areas. As a modification of this 10 process the material may be printed with a composition containing the color discharging agent prior to the application of the ground color which thereupon does not color the printed areas. Both 15 of these methods may be modified by the incorporation in the printing composition of a coloring matter which has an affinity for the materials, or which can be fixed on the material, and which is not affected by the discharging agent. In this manner colored pattern effects may be obtained 20 on colored grounds.

A discharging agent commonly used in the discharge printing of cellulosic materials such as cotton is sodium formaldehyde sulphoxylate. In the discharge printing of materials, made of or 25 containing cellulose acetate, however, sodium formaldehyde sulphoxylate has been found to be relatively ineffective.

It has now been found that excellent discharges 30 on textile materials in general, and on materials made of or containing cellulose acetate or other cellulose esters or ethers in particular, may be obtained with the aid of aldehyde or ketone sulphoxylates of metals capable of exhibiting more than one valency or with the aid of mixtures 35 comprising aldehyde or ketone sulphoxylates and compounds of metals capable of exhibiting more than one valency.

Examples of metals capable of exhibiting more 40 than one valency of which the aldehyde or ketone sulphoxylates may be prepared in accordance with the present invention are tin, titanium, copper and iron. In the production of discharge effects, however, it is preferred to employ the aldehyde or ketone sulphoxylates or other compounds of metals forming colorless or substantially colorless oxidation products, and from this point of view compounds of titanium and tin are preferable to compounds of iron or copper.

The aldehyde and ketone sulphoxylates of 45 metals capable of exhibiting more than one valency may be conveniently obtained by the interaction of aldehyde or ketone sulphoxylates, or materials capable of yielding aldehyde or ketone sulphoxylates, and a compound of the 50 metal. For instance sodium or other alkali metal

formaldehyde sulphoxylates may be treated in aqueous solution with an aqueous solution of a water-soluble stannous, ferrous or titanous salt and the desired metal aldehyde sulphoxylate isolated.

5 The sulphoxylate compound may be derived from any desired aldehyde or ketone. Examples of such bodies are formaldehyde, acetaldehyde, benzaldehyde and acetone. The aldehyde and ketone sulphoxylates obtained in the manner described above may be utilized for the production 10 of discharge effects on textile materials, if requisite after admixture with thickening agents to fit them for local application by printing or the like. It is not essential however to isolate 15 the aldehyde or ketone sulphoxylate compounds as the crude mixtures resulting from the interaction of aldehyde or ketone sulphoxylates and salts of metals capable of exhibiting more than one valency may be directly utilized for the production 20 of discharge effects. Further as previously explained aldehyde or ketone sulphoxylates may be simply mixed with compounds of metals capable of exhibiting more than one valency, if requisite together with thickening agents or other 25 additions, and the mixtures utilized for the production of discharge effects. For example a discharge composition may be employed in accordance 30 with the present invention comprising stannous chloride and sodium formaldehyde sulphoxylate.

The foregoing metal aldehyde and ketone sulphoxylates or mixtures are powerful reducing agents, and, as has been stated, are particularly valuable for the production of discharge effects 35 on textile materials, and particularly on textile materials made of or containing cellulose acetate, cellulose formate, cellulose propionate, cellulose butyrate, or other organic ester of cellulose, or ethyl cellulose, methyl cellulose, benzyl cellulose, 40 or other cellulose ether. They may also be employed with advantage for the production of discharge effects on mixed materials containing organic derivatives of cellulose and other fibres, or on cotton, silk, wool or regenerated cellulose 45 or other textile materials. The compounds may be employed for the production of white discharges, or they may be employed in admixture with coloring matter resistant thereto and having an affinity for or capable of being fixed on the 50 materials for the production of colored discharges, e. g. the insoluble metal compounds of leuco vat dyes described in U. S. application S. No. 605,115 filed April 13, 1932 corresponding to British application No. 14728/31 filed 55 19th

May, 1931. In applying the new process the materials may either first be colored and then the discharge composition applied or the material may first be printed with the discharge composition and the ground color then applied whereupon the latter does not develop in the printed areas.

The discharge compositions employed may contain in addition to the discharging agent or discharging mixture other substances, for example thickening agents, swelling or penetrating agents for the material under treatment, e. g. alcohols, phenols, or hydroquinone in the case of cellulose esters or ethers, and catalysts, e. g. anthraquinone. 10 none. After the application of the discharging preparations the material may be steamed, aged or otherwise treated to effect or complete the discharging action and/or to fix any coloring matters simultaneously applied.

20 The following examples illustrate the invention without being in any way limitative:—

*Example 1*

A cellulose acetate material is dyed with 25 4-nitro-2-methoxy-benzene-azo-dimethyl-aniline, and printed with a freshly prepared printing paste containing:—

|                                 | Parts |
|---------------------------------|-------|
| Sodium formaldehyde sulfoxylate | 10    |
| Methylated spirits              | 10    |
| Gum arabic 1:1                  | 50    |
| Water                           | 22.5  |
| Stannous chloride crystals      | 7.5   |
|                                 | 100.0 |

35 It is then dried, aged for 5 minutes or longer in a Mather and Platt ager, washed, soaped and dried. A good white discharge is obtained on a red ground.

40

A cellulose acetate material is dyed a violet shade with the dyestuff obtained by diazotizing 45 5-nitro-2-amino-anisol and coupling with  $\omega$ -oxyethyl- $\alpha$ -naphthylamine, and is printed with a freshly prepared printing paste having the following composition:—

|                                 | Parts |
|---------------------------------|-------|
| Sodium formaldehyde sulfoxylate | 10    |
| Methylated spirits              | 10    |
| Gum arabic 1:1                  | 50    |
| Water                           | 13.5  |
| Titanous chloride (20% soln.)   | 16.5  |
|                                 | 100.0 |

55 After printing, the material is dried, aged for 5 minutes in a Mather and Platt ager, and then washed, soaped and dried when a good white discharge on a violet ground is obtained.

*Example 3*

The calculated quantity of an aqueous solution of stannous chloride is added to a 10% solution of sodium formaldehyde sulfoxylate and the mixture stirred vigorously and the precipitate which is obtained is pressed out to a 30% concentration, and then mixed with an equal weight of gum arabic thickening. A cellulose acetate material dyed with Dispersol Yellow 3G, is then printed with this composition, and then dried, aged for 5 minutes or more in a Mather and Platt ager, washed, soaped and dried. A good white discharge is obtained on a yellow ground.

What I claim and desire to secure by Letters 15 Patent is:—

1. Process for the production of pattern effects on textile materials containing an organic derivative of cellulose, which comprises locally discharging a dyestuff thereon by means of a titanous 20 aldehyde sulphoxylate.

2. Process for the production of pattern effects on textile materials containing organic derivatives of cellulose, which comprises locally discharging a dyestuff thereon by means of compounds selected from the group of titanous aldehyde and ketone sulphoxylates.

3. Process for the production of pattern effects on textile materials containing cellulose acetate, which comprises locally discharging a dyestuff 30 thereon by means of compounds selected from the group of titanous aldehyde and ketone sulphoxylates.

4. Process for the production of pattern effects on textile materials containing cellulose acetate, 35 which comprises locally discharging a dyestuff thereon by means of titanous formaldehyde sulphoxylate.

5. Discharge compositions suitable for use on materials comprising an organic derivative of 40 cellulose, said compositions containing a compound selected from the group of titanous aldehyde and ketone sulphoxylates.

6. Discharge compositions suitable for use on materials comprising cellulose acetate, said compositions containing a compound selected from 45 the group of titanous aldehyde and ketone sulphoxylates.

7. Discharge compositions suitable for use on materials comprising an organic derivative of 50 cellulose, said compositions containing titanous aldehyde sulphoxylates.

8. Discharge compositions suitable for use on materials comprising cellulose acetate, said compositions containing titanous aldehyde sulphoxylates.

GEORGE HOLLAND ELLIS.